

# UNITED STATES PATENT OFFICE.

RODOLPHE PECHKRANZ, OF CAROUGE-GENEVA, SWITZERLAND.

## PROCESS FOR THE MANUFACTURE OF METALLIC DIAPHRAGMS OF ELECTROLYTIC CELLS.

1,388,754.

Specification of Letters Patent. Patented Aug. 23, 1921.

No Drawing.

Application filed June 1, 1920. Serial No. 385,715.

To all whom it may concern:

Be it known that I, RODOLPHE PECHKRANZ, engineer, a citizen of Switzerland, residing at Carouge-Geneva, Canton of Geneva, in the 5 Confederation of Switzerland, have invented certain new and useful Improvements in Processes for the Manufacture of Metallic Diaphragms of Electrolytic Cells, of which the following is a specification.

10 The present invention relates to the manufacture of metallic bodies and in particular of metal diaphragms for electrolytic cells; and it contemplates the production of a thin, porous diaphragm constructed of a metal—nickel, for instance, or some other metal of the same group—which is inert in respect of the chemical reactions of the particular electrolyte to be used in the cell.

In carrying out the invention, a suitable 20 foundation or support is first treated to form a matrix for the diaphragm, the surface of the matrix being provided at a multitude of points with fine particles of electrical insulating material, after which such surface is oxidized. The support so treated is then 25 placed in an electrolytic bath through which a current is caused to pass, so as to effect the deposit, galvanoplastically, of a coat of nickel upon the prepared surface of the 30 matrix; and at the conclusion of the operation the coating or layer is stripped from the matrix, which can readily be done owing to the interposed oxidized layer between the coating and the matrix which prevents the 35 coating and matrix from adhering together.

The detached layer will be found to be covered all over with extremely fine holes which are produced by the particles of insulating material during the formation of the coating, such particles precluding the deposit of the nickel thereon as will be understood. The 40 porosity of the diaphragm can be regulated by varying the character and size of the insulating particles, and the matrix itself

45 can be used repeatedly until worn out.

In preparing the matrix, a number of methods may be adopted. For example, the surface of a copper or other plate may be covered with minute cells by treating it according to the well-known photo-engraving 50 process; and these cells are then filled with suitable insulating enamel by daubing the enamel all over the plate surface, after which the said surface is pumiced, so as to leave 55 bare the metal network between the cells.

The small particles of enamel are retained in their respective cells by means of a coating of nickel which is then deposited electrolytically upon the plate and which, as it increases in thickness, partially closes the 60 cells and thus forms a virtual setting for each individual particle. This completes the matrix, the surface of which is thereupon oxidized in some suitable way; and then the coating of nickel, or other metal of the 65 same group, forming the diaphragm is deposited electrolytically upon the oxidized surface, such nickel coating being quite thin (for instance, a few hundredths of a millimeter) and consequently offering only a 70 slight resistance to the passage of the electrolytic current.

Instead of proceeding as above described, it is possible to construct the matrix by first oxidizing the plate and then spraying uniformly over its oxidized surface a suitable insulating varnish in pulverized condition, the particles of varnish forming the holes in the nickel coating thereafter deposited upon the plate. Or the minute insulating points 75 80 might be produced upon the oxidized surface of the plate by impression; and still other methods of procedure might be adopted.

The invention might also be carried out by treating a textile fabric—for example, 85 cotton, muslin, thread or silk, etc.—in such a way as to convert it from a non-conductor to a conductor of current, and then depositing upon it the coating of nickel or other metal.

I claim as my invention:

1. A process of manufacturing metal diaphragms for electrolytic cells, comprising the steps of depositing electrolytically upon a foundation a coating of a metal which will 95 be inert to the chemical reactions of the electrolyte in the cell in which it is to be used; and then detaching the metal coating from the foundation.

2. A process according to claim 1, in 100 which the metal deposited upon the foundation is one of the nickel group.

3. A process of manufacturing metal diaphragms for electrolytic cells, comprising the steps of depositing a coating of nickel 105 electrolytically upon a suitable foundation; and then detaching the nickel coating from the foundation.

4. A process of manufacturing metal diaphragms for electrolytic cells, comprising 110

the steps of oxidizing the surface of a suitable metal plate; depositing electrolytically upon such oxidized surface a coating of a metal which will be inert to the chemical reactions of the electrolyte in the cell in which it is to be used; and then detaching the metal coating from said plate.

5. A process of manufacturing metal diaphragms for electrolytic cells, comprising the steps of providing upon the surface of a suitable metal plate a multitude of small particles of insulating material; oxidizing said surface; depositing electrolytically upon such oxidized surface a coating of a metal which will be inert to the chemical reactions of the electrolyte in the cell in which it is to be used; and then detaching the metal coating from said plate.

6. A process of manufacturing metal diaphragms for electrolytic cells, comprising the steps of forming a matrix which is provided upon its surface at a multitude of points with fine particles of insulating material; oxidizing the surface of the matrix; depositing electrolytically upon such oxidized surface a coating of a metal which will be inert to the chemical reactions of the electrolyte in the cell in which it is to be used; and then detaching the coating from the matrix.

electrolyte in the cell in which it is to be used; and detaching the coating from the matrix.

80

7. A process of manufacturing metal diaphragms for electrolytic cells, comprising the steps of forming a matrix which is provided upon its surface at a multitude of points with fine particles of insulating material; forming upon the surface of the matrix a layer of relatively-low electrical resistance; depositing electrolytically upon such layer a coating of a metal which will be inert to the chemical reactions of the electrolyte in the cell in which it is to be used; and detaching the coating from the matrix.

35

8. A thin porous diaphragm for electrolytic cells constructed of a metal which is inert to the chemical reactions of the electrolyte in the cell.

40

9. A thin, porous, nickel diaphragm for electrolytic cells.

45

In testimony whereof I affix my signature in presence of two witnesses.

RODOLPHE PECH-KRANZ.

Witnesses:

D. ROD. DE WORSTLINBERG,  
EDW. EMMANNES.